

March 12, 1963

W. H. SMITH

3,081,241

METHOD AND APPARATUS FOR INTRODUCING  
HYDROGEN INTO A STEAM ATMOSPHERE  
Filed Dec. 24, 1959



Inventor:  
William H. Smith,

by James J. Lickiello  
His Attorney.

1

3,081,241

## METHOD AND APPARATUS FOR INTRODUCING HYDROGEN INTO A STEAM ATMOSPHERE

William H. Smith, Burnt Hills, N.Y., assignor to General Electric Company, a corporation of New York

Filed Dec. 24, 1959, Ser. No. 861,968

4 Claims. (Cl. 204—129)

This invention relates to a method of providing hydrogen for a steam atmosphere and more particularly to the method of electrolytically decomposing the water in a high pressure high temperature steam generating equipment, such as for example, the type used in electrical power generation for the production of hydrogen to minimize corrosion.

An important problem which has been in continual association with high temperature high pressure steam generating equipment is that of corrosion. Corrosion of uncoated metal parts increases rapidly with pressures and temperatures, and in modern steam generating equipment, for example, in the range of 1100 to 1500° F. corrosion is an increasing problem. In this and even higher temperature ranges, it has become the practice to use various materials and metals which will not only withstand the temperatures but also be relatively uncorrodible or suitably protected. One of the better metals which has been considered for high temperature steam atmospheres for good strength and wear characteristics has been molybdenum. The use of molybdenum, however, in high temperature steam generating equipment is limited because of the formation of molybdenum trioxide, due to the exposure of molybdenum to oxygen in the system, which is volatile at high temperatures and, therefore, continual corrosion of molybdenum occurs. The designer of high temperature high pressure steam generating equipment is faced with various parameters in steam generating equipment which warrants the use of metals, for example, molybdenum and tungsten for their high strength and other high temperature advantages and, on the other hand, is faced with minimizing corrosion of these metals at the high temperature conditions by the use of suitable coatings or reducing atmospheres.

It is an object of this invention to minimize metal corrosion in a steam power plant generally.

It is a further object of this invention to provide an improved method of introducing a reducing gas atmosphere in steam generating plants utilizing tungsten and molybdenum.

It is a further object of this invention to provide novel means for the generation of hydrogen gas in a steam generating plant employing tungsten and molybdenum parts.

Briefly described one form of this invention includes the generation of hydrogen in the boiler of a steam generating plant by means of electrolytic decomposition of boiler water within a boiler to release hydrogen as a reducing atmosphere.

These and other advantages and features of this invention will be better understood when taken in connection with the following description and the drawing in which:

FIG. 1 is a schematic diagram of the apparatus employed in this invention.

There are various methods of introducing gases, including hydrogen, into a closed container, such as, a steam boiler. In copending application Serial No. 861,779 filed concurrently herewith, now U.S. Letters Patent No. 3,032,386, issued May 1, 1962, and assigned to the same assignee as the present invention, there is disclosed, for example, that hydrogen may be contained in a separate high pressure tank supply and permitted to enter the steam boiler and that various materials, for

2

example, aqueous ammonium may be added to the boiler feed water to liberate hydrogen in the boiler. The high pressure supply source requires extra tanks under high pressure and considerable modulating equipment to control the amount of gas entering the boiler. Large gas losses are also to be expected in the system through leakage, etc. Since cost is such an important problem in steam power generation, the high pressure tank supply of hydrogen is overshadowed by economic factors. Adding materials, such as, aqueous ammonia, etc., also requires separate tanks, separate materials, additional handling means and, therefore, the economic factor also becomes increasingly important. A novel method of introducing hydrogen to a steam boiler is illustrated in FIG. 1, by electrolytic decomposition of water in a boiler.

Referring now to FIG. 1, there is schematically shown an electrolysis system 10 as applied to a steam boiler. Steam boiler 11 is shown to include a boiler wall 12, and water 13 being converted to steam 14. In order to liberate hydrogen by the electrolytic decomposition of water in accordance with the teachings of this invention, a suitable cathode 15, for example, platinum, carbon, copper, etc. is positioned within boiler 11 in water 13. Cathode 15 is electrically connected by means of a suitable connector 16 to a battery 17 or other source of D.C. current with connector 16 being electrically insulated from boiler 12 by means of an insulator 19. An insoluble anode 20, for example, of platinum, carbon etc. is positioned within a chamber 21 and connected to battery 17 by electrical connector 22. Connector 22 is also electrically insulated from chamber 21 by means of an insulator 23. In order to complete the liquid circuit between the anode 20 and cathode 15, the chamber 21 is connected to the boiler by a conduit 24. In this manner the level of water 13 in the boiler maintains a corresponding level in chamber 21 and a boiler water circuit is provided.

The operation of this invention depends on the well known principle of the electrolytic cell. It is generally known that an electrical current can be used to produce hydrogen and oxygen from water by electrolysis. In an electrolytic cell, electrical energy from an outside source serves to produce the chemical changes involved, a small part being wasted as heat. As a typical illustration of the decomposition of water, an electrical current may be passed through water using insoluble electrodes of platinum or carbon. The  $H^+$  ions of the acid will be attracted by the negative plate and repelled by the positive plate and the negative ions will be attracted by the positive and repelled by the negative plate. The result will again be a drifting of ions in both directions through the water. Each  $H^+$  ion on each of the cathode combines with an electron there, forming a hydrogen atom. These atoms combine into molecules and escape as gas, i.e.,  $2H^+ + 2e^- \rightarrow H_2 \uparrow$ . It is understood that while hydrogen is formed or liberated at the cathode, oxygen is being continually given off at the anode. The invention, therefore, as depicted in FIG. 1 is the equivalent of an electrolytic cell. While the water in a steam power plant is generally maintained at a high purity level, where the water is less electrically conductive than desirable, suitable additives may be included therein such that a good electrical circuit is established between the cathode and the anode.

The continual liberation of hydrogen from cathode 15 supplies the necessary quantities of hydrogen to minimize corrosion of metal parts associated with the steam power generating equipment including molybdenum which may be employed in steam turbine buckets and blades. Molybdenum trioxide forms upon exposure of molybdenum to oxygen at high temperatures and is highly

volatile at temperatures of 1000° F. and above and thus is a deteriorating feature. Where the supply of oxygen is diminished,  $\text{MoO}_2$  forms on molybdenum and acts as a protective coating. The principle of this invention, therefore, need not be applied to produce hydrogen in sufficient quantities to act as a reducing atmosphere but only to supply a sufficient or predetermined quantity of hydrogen to a normally oxidizing atmosphere to form the protective coating  $\text{MoO}_2$  on molybdenum instead of  $\text{MoO}_3$  which is highly volatile and deteriorating.

The anode and cathode are not positioned together within the boiler 11 since the decomposition of water will release oxygen into the boiler and minimize the effect to be obtained by the liberation of hydrogen. The provision of the boiler water circuit thereby renders this invention particularly adaptable to enclosed steam power systems, where, due to the fact that oxygen is also liberated, decomposition of boiler water is not contemplated as a means of producing hydrogen. While in the electrolytic cell, oxygen is continually released from the anode, a suitable pressure relief valve 25 is positioned adjacent chamber 21 to be controlled by means well known in the art to maintain the pressure within the system at the desired level and to release oxygen as it is being formed. Hydrogen liberated at the cathode can enter the steam while oxygen liberated anode can be withdrawn and recovered as a useful by-product.

Where other systems of introducing hydrogen in a steam boiler are employed, the embodiment of this invention may be utilized as a make-up supply or an auxiliary to other and different systems. The electrolytic decomposition of water is more particularly applicable as a make-up means for supplying hydrogen where hydrogen is supplied from other sources and where the quantity desired is high. This system is also applicable to other power generating equipment, for example, nuclear reactors employing the boiling water principle, and the various sizes and power requirements of the cell may be varied to suit particular needs.

It can thus be seen that the objects of my invention are obtained by the use of the electrolysis method to decompose boiler water to form hydrogen in steam power generating equipment and that such a method may be used in addition to other present methods. The production of hydrogen limits the formation of volatile  $\text{MoO}_3$  on molybdenum.

While the present invention has been described with reference to a particular embodiment, it will be understood that numerous modifications may be made by those skilled in the art without actually departing from this invention. Therefore, I aim in the appended claims to cover all such equivalent variations as comes within the true spirit and scope of the foregoing disclosure.

What I claim as new and desire to secure by Letters Patent of the United States is:

1. Steam generating apparatus which comprises a boiler, a water chamber connected to said boiler, a cathode positioned in and electrically insulated from said boiler for generating hydrogen gas therein, an insoluble anode positioned in and electrically insulated from said water chamber for generating oxygen gas therein, a source of electric current connected to said anode and said cathode, and oxygen gas relief means provided for said water chamber and adapted to exclude oxygen gas from said boiler.

2. Steam generating apparatus which comprises a boiler, a water chamber, a conduit connecting said boiler to said water chamber, a cathode positioned in and electrically insulated from said boiler and adapted to generate hydrogen gas therein, an insoluble anode positioned in and electrically insulated from said water supply cham-

ber and adapted to generate oxygen gas therein, a source of electric current connected to said anode and said cathode, and oxygen gas relief means provided for said water chamber and adapted to exclude oxygen gas from said boiler.

3. A method of introducing electrolytic hydrogen gas into a steam atmosphere above a steam generating water supply and of introducing electrolytic oxygen gas into an atmosphere above a second water supply which comprises providing a steam generating water supply in a boiler, providing a second water supply in a chamber, providing a third water supply connecting said first water supply and said second water supply, providing an electrode in said first water supply, insulating electrically said electrode from said boiler, decomposing electrolytically a portion of said first water supply whereby only electrolytic hydrogen gas is generated in said first water supply and liberated into said steam atmosphere to limit oxidation of metals exposed to said steam atmosphere, providing an electrode in said chamber, insulating electrically said electrode from said chamber, decomposing electrolytically a portion of said second water supply whereby only electrolytic oxygen gas is generated in said second water supply, and removing said oxygen gas from said second water supply, thereby preventing mixing of said oxygen gas with said hydrogen gas.
4. A method of introducing electrolytic hydrogen gas into a steam atmosphere above a steam generating water supply and of introducing electrolytic oxygen gas into an atmosphere above a second water supply which comprises providing a steam generating water supply in a boiler, providing a second water supply in a chamber and connected to said first water supply, providing an electrode in said first water supply, insulating electrically said electrode from said boiler, decomposing electrolytically a portion of said first water supply whereby only electrolytic hydrogen gas is generated in said first water supply and liberated into said steam atmosphere to limit oxidation of metals exposed to said steam atmosphere, providing an electrode in said chamber, insulating electrically said electrode from said chamber, decomposing electrolytically a portion of said second water supply whereby only electrolytic oxygen gas is generated in said second water supply, and removing said oxygen gas from said second water supply, thereby preventing mixing of said oxygen gas with said hydrogen gas.

#### References Cited in the file of this patent

#### UNITED STATES PATENTS

|    |           |               |                |
|----|-----------|---------------|----------------|
| 50 | 736,868   | McCarty       | Aug. 18, 1903  |
|    | 800,296   | Harris et al. | Sept. 26, 1905 |
|    | 1,581,944 | Hausmeister   | Apr. 20, 1926  |
|    | 1,666,523 | Bailey        | Apr. 17, 1928  |
| 55 | 1,783,726 | Lappe et al.  | Dec. 2, 1930   |
|    | 1,825,477 | Reichart      | Sept. 29, 1931 |
|    | 1,835,425 | Pier          | Dec. 8, 1931   |
|    | 1,912,188 | Gann          | May 30, 1933   |
|    | 2,763,611 | Breden        | Sept. 18, 1956 |

#### FOREIGN PATENTS

|    |         |               |               |
|----|---------|---------------|---------------|
| 60 | 104,856 | Germany       | Mar. 30, 1898 |
|    | 14,818  | Great Britain | July 7, 1900  |
|    | of 1898 |               |               |
| 65 | 154,610 | Great Britain | Nov. 24, 1921 |
|    | 583,449 | Great Britain | Dec. 18, 1946 |
|    | 610,725 | Great Britain | Oct. 20, 1948 |

#### OTHER REFERENCES

- Fox: Corrosion Technology, December 1955, pages 70 375-6.